

## UNITED STATES PATENT OFFICE

2,103,018

PROCESS FOR ENHANCING THE STABILITY  
TO WATER OF EFFECTS PRODUCED ME-  
CHANICALLY ON TEXTILES CONTAINING  
CELLULOSEAndreas Ruperti, Basel, Switzerland, assignor to  
Society of Chemical Industry in Basle, Basel,  
SwitzerlandNo Drawing. Application March 23, 1936, Serial  
No. 70,540. In Switzerland March 28, 1935

8 Claims. (Cl. 8-20)

It is known practice to produce mechanically on textiles containing cellulose effects such as are obtainable, for example, by the action of pressure, if desired in conjunction with heat, as is the case in the treatment with an embossing calender. Such effects, however, are only stable so long as they do not come into contact with water. If the impressed textile is washed or exposed to rain or to a moist atmosphere, the effect 10 is more or less completely lost.

This invention relates to a process by which the resistance of these effects to the action of water may be increased in a surprising manner by conversion of the cellulose into a cellulose derivative which in comparison with the original cellulose has a diminished capacity for swelling in water, in the sense that not only a moist atmosphere or rain, but also hot washing, dyeing and like treatments, have a diminished tendency to injure the effect. In this manner results are obtained which hitherto could not be achieved except in a complicated manner during weaving.

The effects in question may be produced by any known process, for example by stamping, pressing, ironing or the like.

As parent materials there may be used textiles which consist of or contain native cellulose of any origin, whether pretreated or not, for instance cotton, mercerized cotton, ramie, flax, hemp or the like, or of regenerated cellulose, for instance viscose, cuprammonium cellulose, de-nitrated cellulose, cellulose obtained by precipitation of solutions of cellulose in quaternary ammonium salts, and native and regenerated cellulose, or cellulose, native or regenerated, and other fibers. The parent materials most important are piece-goods or knitted goods; for certain purposes loose material or thread may be used. The parent material may be undyed or may have been previously dyed with a dye-stuff stable to the treatment.

For converting the cellulose into the cellulose ester which, in comparison with the original cellulose, as described above, has a diminished capacity for swelling in water, there may be used any known esterifying agents and methods which esterify cellulose with retention of the structure. These methods are well known and some of these are for example described in the specification No. 1,930,895 or 1,922,287, or in the German Patents No. 224,330, 347,130, 380,994 or 525,084. These methods make it possible to esterify cellulose without causing dissolution or swelling the material too much.

In the case of esterifying processes which em-

brace as a part of the operation a treatment having a swelling effect on cellulose, for example, a treatment in aqueous solution, the desired effects must be produced after this part of the operation.

The esterification can be carried out in a suitable apparatus with the aid of a suitable acylating agent, for example an acid anhydride, such as acetic anhydride, propionic anhydride, butyric anhydride, valerianic anhydride, isovalerianic anhydride, monochloroacetic anhydride, phthalic anhydride, or with an acid chloride, such as acetyl chloride, propionyl chloride, butyryl chloride, palmityl chloride, stearoyl chloride, benzoyl chloride, in presence or absence of an alkaline catalyst, such as sodium acetate, potassium acetate, potassium carbonate or potassium sulfite, or of a neutral or acid catalyst, such as sulfuric acid, zinc chloride, copper sulfate; and in presence or absence of a solvent or diluent, such as benzene, benzine, xylene, chlorobenzene, perchlorethylene, pyridine, with or without preliminary swelling of the material, for instance with a base, an acid or a concentrated solution of salt; or with a suitable etherifying agent, such as benzyl chloride; in either case the treatment must not destroy the structure of the parent material.

When piece-goods are under treatment, the process is advantageously conducted as a continuous operation.

The cellulose constituents of the material produced differ in their behaviour in the matter of dyeing from the parent material, in that they have an enfeebled or no affinity for direct-, vat- and sulfur-dyestuffs, whereas they can be dyed more or less strongly with the usual dyestuffs for artificial silk.

The following examples illustrate the invention:

## Example 1

Viscose satin or crêpe satin piece-goods are impregnated with a solution of potassium acetate of 50 per cent strength, dried, pressed on an embossing calender with a fancy pattern and treated for half-an-hour at 90° C. with a solution of 5 per cent of acetic anhydride in benzine. The esterifying liquid is sucked off, or simply drained off, whereupon the acetylated material is dried with recovery of the volatile constituents of the treating liquor which still adhere to it. It is then washed with water and dyed with an acetate silk dyestuff in a manner usual for dyeing acetate silk. The embossed effect remains

5

10

15

20

25

30

35

40

45

50

55

through all these operations and is completely stable to water and washing. In like manner a durable imitation crêpe may be produced by embossing an artificial silk fabric impregnated with 5 potassium acetate and subsequently acetylated.

*Example 2*

Cotton piece-goods are passed through an embossing calender and treated for 3 hours at 50° C. 10 with 15 times their weight of a solution of 30 per cent strength of acetic anhydride in glacial acetic acid in presence of zinc chloride amounting to 1 per cent by weight of the solution. After separating the adhering acetylating liquor the 15 goods are washed with water and dried. The embossed effect remains, even when the goods are subsequently dyed or washed.

*Example 3*

20 Cotton piece-goods are folded and pressed hot so that a pleating effect is produced. The goods are then treated with 10 to 15 times their weight of a solution of 10 per cent strength of benzoyl chloride in pyridine for half-an-hour at 80° C., 25 and then washed with water and dried. A pleating effect stable to water is produced.

What I claim is:—

1. A process for enhancing the stability to water of effects unstable to water produced locally by 30 mechanical means on textiles containing cellulose, which consists in esterifying the cellulose, after the effect has been produced, with retention of the structure of the cellulose.

2. A process for enhancing the stability to water 35 of effects unstable to water produced locally by mechanical means on textiles containing cellulose, which consists in esterifying the cellulose, after the effect has been produced, with an aliphatic acid anhydride in the presence of a potassium salt of a weak acid.

3. A process for enhancing the stability to water of effects unstable to water produced locally by 5 mechanical means on textiles containing cellulose, which consists in esterifying the cellulose, after the effect has been produced, with an aliphatic acid anhydride in the presence of a potassium salt of a weak aliphatic acid.

4. A process for enhancing the stability to water of effects unstable to water produced locally by 10 mechanical means on textiles containing cellulose, 10 which consists in esterifying the cellulose, after the effect has been produced, with acetic anhydride in the presence of potassium acetate.

5. A process for enhancing the stability to water of effects unstable to water produced locally by 15 mechanical means on cotton, which consists in esterifying the cotton, after the effect has been produced, with an aliphatic acid anhydride in the presence of a potassium salt of a weak aliphatic acid.

6. A process for enhancing the stability to water of effects unstable to water produced locally by 20 mechanically means on cotton, which consists in esterifying the cotton, after the effect has been produced, with acetic anhydride in the presence 25 of potassium acetate.

7. A process for enhancing the stability to water of effects unstable to water produced locally by 30 mechanical means on regenerated cellulose, which consists in esterifying the regenerated cellulose, 30 after the effect has been produced, with an aliphatic acid anhydride in the presence of a potassium salt of a weak aliphatic acid.

8. A process for enhancing the stability to water of effects unstable to water produced locally by 35 mechanical means on regenerated cellulose, which consists in esterifying the regenerated cellulose, 35 after the effect has been produced, with acetic anhydride in the presence of potassium acetate.

ANDREAS RUPERTI. 40